

## UNITED STATES PATENT OFFICE

2,589,973

## LUBRICATING GREASE COMPOSITION

Paul V. Smith, Jr., Westfield, and Arnold J. Morway, Rahway, N. J., assignors to Standard Oil Development Company, a corporation of Delaware

No. Drawing. Application November 1, 1949,  
Serial No. 124,942

19 Claims. (Cl. 252—41)

1

This invention pertains to lubricating grease compositions of improved structural stability containing hydroxy ether acid soaps. It relates also to a process of preparing grease compositions which are structurally stable.

The invention particularly concerns lubricating greases which employ as a thickening agent the alkali, alkaline earth, or aluminum metal soaps of branched chain hydroxy ether aliphatic acids of the general formulas:



and



or



where  $\text{R}_1$  and  $\text{R}_2$  are aliphatic hydrocarbon groups of 3 to 12 carbon atoms each, preferably, but not necessarily saturated,  $\text{R}_3$  is an aliphatic hydrocarbon group of 2 to 6 carbon atoms, and  $m$  is an integer of at least 1, preferably 1 to 2 or 1 to 3. Preferably,  $\text{R}_1$  and  $\text{R}_2$  are 6 to 10 carbon atoms each and they total about 14 to 18 carbon atoms.  $\text{R}_3$  contains preferably 2 to 3 carbon atoms. The acid thus contains preferably from 16 to 24 carbon atoms, about 20 being specifically preferred. It will be noted that the  $\text{O}-\text{R}_3$  radical in the side chain may be repeated 2 to 3 times, or even more.

In particular, an acid of formula



i. e., the ether of 12 hydroxy stearic acid, is found to be an especially suitable material for forming the soap, but the entire class of homologous saturated acids, within the limits of chain length mentioned above, may be employed. Derivatives of certain unsaturated acids, such as ricinoleic, may also be used. Among the specific compounds

2

which may be employed are 8-( $\beta$ -hydroxy-ethoxy)-stearic acid, 12-( $\beta$ -hydroxy-ethoxy)-stearic acid, 12-( $\beta$ -hydroxy- $\alpha$ -propoxy)-ricinoleic acid, 10-( $\beta$ -hydroxy-isobutoxy)-palmitic acid, mixed hydroxy-alkyl ether derivatives of hydroxy acids prepared by chlorinating fatty acids and hydrolyzing the chloro acids, etc.

In order to produce the branched chain hydroxy ether acids mentioned above, the following method may be pursued. Hydroxy acids, for example those of natural occurrence, such as ricinoleic (hydroxy stearic) acid, may be reacted with an olefin oxide such as ethylene oxide or propylene oxide. The reaction may be carried out without a catalyst, but it is preferable to use a Friedel-Crafts catalyst such as  $\text{BF}_3$ ,  $\text{SnCl}_4$ , or the like.

For example, 0.1 mol (30 g.) of hydroxy stearic acid was dissolved in toluene containing 0.5 ml. of  $\text{SnCl}_4$ . The mixture was stirred rapidly in a 20 3-necked flask while 20 g. (0.45 mol) of ethylene oxide was bubbled in. The reaction temperature was kept between 50° and 60° C. The solvent was removed by keeping the flask in a steam bath for several hours. The remaining product, which 25 solidified on cooling, was analyzed for acid and found to have an acid value of 0.211 centi-equivalents per gram, corresponding to better than a 95% purity of acid. The small non-acidic residue probably was toluene. With longer treatment on the steam bath, the acid may be made practically 100% pure.

Other hydroxy acids, both aliphatic and aromatic, appear to react similarly. The production of the hydroxy ether acids per se forms no part 35 of the present invention but it may be noted that the process just described appears to be applicable to various hydroxy fatty acids and to aromatic acids such as salicylic acid, and the like. The former may be said to have the general formula mentioned above. The branched chain aliphatic acids of fairly high molecular weight are 40 the ones of interest in grease manufacture.

It is particularly to be noted that the alkylene oxide radical may occur only once or it may be 45 repeated twice or more. In general, the acids actually produced in practice are a mixture of branched chain compounds having, respectively, one alkylene ether and two or even more alkylene ether groups. Acids with more than two such 50 groups in series appear to be present in very limited quantities, if at all, under the reaction conditions described above, but under other conditions they may appear in substantial proportions.

The properties of greases containing the soaps

of these various products are undoubtedly affected by the number of alkylene oxide radicals in series. The invention includes the various reaction products just mentioned and, in particular, greases containing soaps of acids at least with 1 to 2 and in some cases, more alkylene oxide groups.

The specific formulas of the reaction products of olefin oxides and hydroxy acids may be written in several ways, including those given above. The products may take the formula



where  $\text{R}_1$  and  $\text{R}_2$  have the same meaning as above and where  $\text{R}_3$ ,  $\text{R}_4$ ,  $\text{R}_5$  and  $\text{R}_6$ , or any of them, may be either hydrogen or a methyl group. This alkylene-oxide group may occur only once or more than once, e. g., twice or more. Hence,  $m$  is an integer whose value may be 1, 2, 3, or even more, but usually 1 or at most 2.

The branched chain hydroxy ether acids just described may be converted to soaps by using the appropriate metal oxide, hydroxide, or carbonate, as will be obvious to those skilled in the art. The alkali metal soaps, especially the lithium soaps, of such acids, are particularly meritorious, but the calcium, barium and aluminum soaps also may be used, and indeed the metals in general. These soaps may be mixed with each other and/or may be used in admixture with conventional soaps, e. g., the alkali or alkaline earth metal, or aluminum soaps of straight chain fatty acids. In addition, conventional salts and/or soaps of low molecular weight, such as alkali or alkaline earth metal acetates, acrylates, propionates, furoates, and the like, may also be included in the ingredients. The combination of low molecular weight salts with soaps of higher molecular weight is often advantageous, as is now well-known in the art.

Soaps of the type characterizing the present invention may be used (alone or in combination with other and conventional thickeners, as mentioned above) to prepare greases of mineral lubricating oils, synthetic oils, or mixtures thereof. The following detailed examples show lithium and calcium soaps used in various oils and combinations of oils, but the invention clearly is not limited to the lithium and/or calcium base greases or to the specific lubricants claimed. The improvement in stability and other characteristics of lithium soap greases is noteworthy, and this is a preferred product.

The proportions of ingredients used may be varied within usual limits, although it should be noted that somewhat smaller quantities of the branched chain hydroxy ether acid soaps of this invention may be required in some case to thicken a grease to a given consistency than is required of conventional soaps. As little as about 3% of the new type soaps, or as much as 35% to 40%, based on the weight of the total composition, may be used. According to the present invention, the new soaps may be used alone or they may be combined with conventional soaps. In the latter case, the hydroxy ether acid soap preferably should comprise at least one-third of the total soap. Hence, a grease composition of the present invention will comprise at least 1%, up to a maximum of about 40% by

weight, of hydroxy ether acid soap, with a total soap content of 3 to 40%. Preferred ranges are 6 to 20% total soap, which preferably includes not less than 2% of the hydroxy ether acid soap and at least 4% of additional thickener, the latter being either the same or some conventional soap.

In the specific case of lithium soap greases, the use of about 8 to 12% total soap is particularly preferred, at least one-third of which soap is of hydroxy ether acid. Where firm consistency is desired with minimum soap consumption (the lithium soaps being relatively expensive) a combination of about equal parts of conventional lithium soap (e. g., lithium stearate) and the hydroxy ether acid soap is particularly desirable. In the case of calcium greases, somewhat higher quantities, e. g., 20% or more of soap, appear to be preferable.

As suggested above, the present invention includes not only a new composition but an improved process of preparing a composition having excellent properties of stability resistance to moisture, and the like. A grease is prepared, preferably by adding 1 to 40 parts by weight of the branched chain hydroxy ether acid (containing one or more alkylene oxide groups) to 10 to 96 parts by weight of mineral base lubricating oil. The mixture of oil and acid is next heated moderately with stirring to a temperature between 100° and 200° F., for example 150° F. At this point, an aqueous solution of a saponifying agent, such as lithium hydroxide, sodium hydroxide, calcium hydroxide, or the like, is added in suitable quantity to neutralize the acid. An aqueous solution of lithium or calcium hydroxide, for example, is added at the temperature of about 150° F.

The mixture is next heated to a temperature of at least 212° F., and preferably a little higher, to dehydrate the grease and thereafter the temperature is further raised to cook the grease and form a grease structure. The cooking temperature is between 300° and 500° F., about 400° F. being preferred. During the various steps just described, the product is continuously stirred, preferably with a mechanical stirrer.

After cooking, the grease is cooled in thin layers, either in a close clearance mechanical cooler or by pouring into thin layers in cooling pans or drum chilling. Thereafter, the product is homogenized and packaged.

Where it is desired to prepare a grease having extremely good temperature characteristics, for example, a grease to be used both at very low and very high temperatures as in the lubrication of airplane instruments, it may be preferable to use a substantial quantity of a synthetic oil, such as di-2-ethylhexyl sebacate or the tri-ethylene glycol ester of 2-ethylhexanoic acid, or other related branched chain esters having outstanding temperature viscosity characteristics. Where such lubricants are to be used, it is preferred to prepare the soap in mineral oil, as described above, adding the synthetic oils after cooking to avoid hydrolysis of the esters. The proportions of mineral oil and ester oil may be varied, but preferably at least 10% of the composition should be of mineral base oil. Aside from requirements for high and low temperature operation, the mineral base greases are quite satisfactory in themselves.

If it is desired to prepare a lubricant which contains no mineral base oil, a preformed soap should be used and dispersed thoroughly into

the synthetic oil so as to obtain a good grease structure. This may be done by methods well-known in the art. Conventional greases, prepared either by forming the soaps of straight chain fatty acids in situ or prepared from pre-formed soaps, are commonly deficient in structural stability especially when subjected to heavy mechanical working. Greases prepared according to the method described above are superior in this respect.

Thus, conventional lithium base greases prepared by forming the lithium soap of stearic acid, hydrogenated fish oil acids, and the like, in lubricating oil are structurally unstable to long and severe mechanical working. This instability is readily shown by working the grease in the standard ASTM grease worker for about 1000 strokes. The conventional lithium soap greases break down into a semi-fluid product under this treatment.

On the other hand, greases prepared from the lithium soaps of hydroxy fatty acids, such as hydroxy stearic acid, wherein the hydroxy group is attached directly to the main and only hydrocarbon chain, have good structural stability but they tend to harden under high shearing stresses. They also possess comparatively poor water resisting characteristics.

According to the present invention, greases prepared from hydroxy ether acids of the type described above, have both good structural stability to mechanical working and a good resistance to water. They do not harden under high shearing stresses.

As another feature of the present invention, it is found that the combination of the soaps of hydroxy ether acids with conventional soaps yields a grease of firmer consistency for a given quantity of soap than the conventional products. Where mixed soaps are so used, as previously mentioned, the hydroxy ether acid soap should comprise at least about one-third of the total soap employed. Better results are obtained if approximately equal quantities of conventional or straight chain soap such as lithium stearate and the soap of the present invention are combined.

The invention will be more fully understood by reference to the following examples:

*Example I*

10.00% hydroxy ether acid of invention of molecular weight about 363 (derived from ethylene oxide treatment of 12-hydroxy stearic acid)

1.23% LiOH·H<sub>2</sub>O

68.77% di-2-ethylhexyl sebacate

20.00% refined coastal type mineral oil of 37 S. U. S. viscosity at 210° F.

The hydroxy ether acid evidently was a mixture of products containing a single ethylene oxide radical and two, or possibly more, ethylene oxide radicals in series. It was added to the cold mineral oil and charged to a fire heated grease kettle. The mixture was next warmed to 150° F. while agitating. The lithium hydroxide, dissolved in boiling water, was next added to neutralize the acid and form the soap in mineral oil. After the mass was dehydrated (225° F.), the ester constituent was added and the grease further heated to 400° F. The hot molten grease was then poured onto a drum chiller for quick cooling. The molten grease on cooling was collected by scraping from the

chiller and homogenized by stirring in a cold grease kettle or passing through a Cornell homogenizer. The product was of stable structure and had a very good texture.

5 Properties:

|                                                     |      |
|-----------------------------------------------------|------|
| Free alkalinity (as LiOH) %                         | 0.10 |
| ASTM worked penetration, 77° F., mm./10             | 250  |
| Penetration after working 10,000 strokes            |      |
| ASTM worker employing fine hole worker plate mm./10 | 297  |
| Dropping point °F.                                  | 358  |
| Appearance—Excellent, smooth, buttery structures.   |      |

*Example II*

|                                                          |  |
|----------------------------------------------------------|--|
| 8.00% acid of invention, as in Example I                 |  |
| 1.00% LiOH·H <sub>2</sub> O                              |  |
| 10.00% coastal type material oil of 40 S. U. S.          |  |
| 20. viscosity at 210° F.                                 |  |
| 81.00% tri-ethylene glycol ester of 2-ethylhexanoic acid |  |

Prepared in similar manner as shown in Example I. The grease was of a soft consistency having a worked penetration of 350 mm./10 and a dropping point of 326° F.

*Example III*

|                                                                                                                                                                                                                                         |     |
|-----------------------------------------------------------------------------------------------------------------------------------------------------------------------------------------------------------------------------------------|-----|
| 30 Equal portions of the two greases prepared above were mixed and heated to 400° F. The hot molten grease at 400° F., was poured into pans in shallow layers and cooled. After cooling, the grease was of excellent, smooth structure. |     |
| Worked penetration at 77° F., mm./10                                                                                                                                                                                                    | 310 |
| Dropping point °F.                                                                                                                                                                                                                      | 344 |

*Example IV*

|                                                                                                              |  |
|--------------------------------------------------------------------------------------------------------------|--|
| 40 8.0% preformed dry lithium soap of invention, as in Example I, but formed without presence of mineral oil |  |
| 92.0% low cold test mineral oil of 70 S. U. S. viscosity at 210° F.                                          |  |

|                                                                                                                                                                                                                                          |  |
|------------------------------------------------------------------------------------------------------------------------------------------------------------------------------------------------------------------------------------------|--|
| 45 The dry soap was slurried with the mineral oil and heated to 400° F. The grease on cooling relatively rapidly in thin layers was of excellent soft smooth structure which tended to become semi-fluid on extended mechanical working. |  |
| 50                                                                                                                                                                                                                                       |  |

*Example V*

|                                                           |  |
|-----------------------------------------------------------|--|
| 55 5.00% lithium stearate                                 |  |
| 5.00% lithium soap of acid of invention, as in Example IV |  |
| 90.00% mineral oil as in Example IV.                      |  |

60 The combined soaps were dispersed in the mineral oil at 420° F. and cooled. By either rapid cooling (thin layers in cooling pans) or slow cooling, an excellent smooth grease was obtained.

|                                                                                                                                        |     |
|----------------------------------------------------------------------------------------------------------------------------------------|-----|
| 65 Worked penetration, 60 strokes, 77° F., mm./10                                                                                      | 295 |
| Penetration after 10,000 strokes in worker employing fine hole worker plate, 77° F., mm./10                                            | 325 |
| Dropping point °F.                                                                                                                     | 365 |
| Bearing test—No tendency to change smooth, short-fibre structure at 200–225° F. to a fibrous rubbery form which throws out of bearing. |     |

70 A few experiments have been run also to determine the effectiveness of the calcium soaps as thickeners for mineral oil and esters.

An acid, derived by treating 12-hydroxy stearic acid with ethylene oxide and having a molecular weight of 363 was employed. The following greases were prepared.

*Example VI*

20.00% hydroxy-ether acid  
2.30% hydrated lime  
77.30% naphthenic-type oil of about 100 S. U. S. viscosity at 100° F., and 40 S. U. S. at 210° F.

The acid and 80% of the oil were heated together until the acid had melted and dispersed in the oil (about 150° F.). The lime was slurried in the balance of the oil and added to oil-acid dispersion while agitating. A solid grease composition was formed of excellent structure stability, but somewhat grainy in appearance.

*Example VII*

20.00% hydrofol acids "54" (hydrogenated fish oil acids)—Stearic acid could be used instead.  
3.00% hydrated lime  
77.00% mineral oil as in Example VI

Prepared similar to above Example VI.

*Example VIII*

The two greases of Examples VI and VII were mixed together in equal proportions and heated to 250–260° F. (Grease fluidized at 275° F.). On cooling, an excellent smooth grease of excellent structure stability was formed of about 220 mm./10 penetration.

Dropping point, 288° F.

Boiling water test—10 grams of grease placed in boiling water for 3 hours. No disintegration or separation of the grease. No cloudiness in water.

In preparing greases according to this invention, the particular metal oxide or hydroxide used for saponification should be selected that is most suitable for the intended purpose. The lithium and calcium base greases have good water resistance. Lithium greases show superior stability but of course the calcium greases are less expensive. Soda base greases may readily be prepared in the same manner but they are less water resistant. Mixed base greases of these and other metals also may be prepared.

While the foregoing examples all relate to the lithium and the calcium soaps, some of which are commonly more difficult to prepare than the more conventional metal base products, it will be understood that various other metal bases will be used with equal facility and with comparable beneficial results. It will also be understood that conventional additives may be included in the grease compositions without altering their basic properties. Thus, the usual anti-oxidants, corrosion inhibitors, tackiness agents, extreme pressure compounds, and the like, may be included, as will be obvious to those skilled in the art.

What is claimed is:

1. A lubricating grease composition consisting essentially of lubricating oil thickened to a grease consistency with 3 to 40% by weight, based on the total composition, of metal soap of aliphatic carboxylic acid, said metal soap comprising at least one-third part of a soap of an acid having the general formula



wherein R<sub>1</sub> and R<sub>2</sub> are alkyl groups of 3 to 12

carbon atoms each and R<sub>3</sub> is an alkyl group of 2 to 6 carbon atoms.

2. A lubricating grease composition consisting essentially of a lubricating oil thickened to a grease consistency with 3 to 40% of soap of aliphatic carboxylic acid, at least one-third of said soap being a metal soap of branched chain hydroxy aliphatic acid of 18 to 23 carbon atoms, the hydroxy group being on a side chain and the acid radical containing at least one C<sub>2</sub> to C<sub>3</sub> alkylene ether group in a side chain.

3. A lubricating grease composition consisting essentially of a lubricating oil thickened to a grease consistency with a metal soap of aliphatic carboxylic acid, said thickener comprising at least one-third part by weight of a metal soap of a hydroxy ether acid having the general formula



wherein R<sub>3</sub>, R<sub>4</sub>, R<sub>5</sub>, and R<sub>6</sub> are each selected from the class consisting of methyl groups and hydrogen and wherein R<sub>1</sub> and R<sub>2</sub> are each alkyl groups of 3 to 12 carbon atoms, totaling 14 to 18 carbon atoms.

4. Composition according to claim 3, wherein said oil comprises a synthetic ester oil.

5. Composition according to claim 3, wherein said oil is mineral oil.

6. Composition according to claim 3, wherein said soap of hydroxy ether acid is an alkali metal soap.

7. Composition according to claim 3, wherein said soap of hydroxy ether acid is lithium soap.

8. A lubricating grease composition consisting essentially of a lubricating oil thickened to a grease consistency with about 8 to 12% by weight, based on the total composition, of soap of aliphatic carboxylic acid which includes at least one-third part of lithium soap of an acid having the general formula



wherein R<sub>1</sub> and R<sub>2</sub> are alkyl groups of 6 to 10 carbon atoms each, totaling 14 to 18 carbon atoms, n is 2, and m is an integer of 1 to 3.

9. Composition according to claim 2 wherein the metal of the soap is an alkali metal.

10. Composition according to claim 2 wherein the metal of the soap is an alkaline earth metal.

11. Composition according to claim 2 wherein the metal of the soap comprises lithium.

12. Composition according to claim 2 wherein the metal of the soap comprises calcium.

13. Composition according to claim 3, wherein the hydroxy ether acid has the formula



14. Composition according to claim 8, wherein the acid has the formula



15. The process of preparing a stable metal base grease which comprises adding 1 to 40 parts by weight of a branched chain hydroxy ether

saturated aliphatic acid of 17 to 23 carbon atoms and having the hydroxy group on a side chain, to 10 to 96 parts of mineral base lubricating oil, heating to a temperature of 100° to 200° F., adding an aqueous solution of a metal base to saponify said acid in situ in said oil, heating to a temperature of at least 212° F. to dehydrate, adding a synthetic ester oil, further cooking to a temperature of 300° to 500° F. to form a grease structure, and cooling in thin layers.

16. Process according to claim 15, wherein the metal base is lithium hydroxide.

17. Process according to claim 15, wherein the metal base is calcium hydroxide.

18. Composition as in claim 8, wherein the lubricating oil comprises a substantial proportion of di-2 ethylhexyl sebacate.

19. Composition as in claim 8, wherein the lubricating oil comprises a substantial proportion of tri-ethylene glycol ester of 2-ethylhexanoic acid. 20

PAUL V. SMITH, JR.  
ARNOLD J. MORWAY.

## REFERENCES CITED

The following references are of record in the file of this patent:

## UNITED STATES PATENTS

| Number    | Name           | Date           |
|-----------|----------------|----------------|
| 2,435,828 | Guest          | Feb. 10, 1948  |
| 2,435,829 | Guest          | Feb. 10, 1948  |
| 2,436,347 | Zimmer et al.  | Feb. 17, 1948  |
| 2,450,221 | Ashburn et al. | Sept. 28, 1948 |
| 2,457,640 | Bruson et al.  | Dec. 28, 1948  |
| 2,475,589 | Bondi          | July 12, 1949  |

## FOREIGN PATENTS

| Number  | Country       | Date         |
|---------|---------------|--------------|
| 615,182 | Great Britain | Jan. 3, 1949 |